

Aug. 22, 1944.

W. GARNER  
SHOCK-ABSORBING OR CUSHIONING MATERIAL  
MADE FROM FIBROUS SUBSTANCES  
Filed Aug. 9, 1943

2,356,456

Fig. 1.



Fig. 2.



Fig. 3.



Attwactor:  
Walter Garner  
By his attorneys,  
Baldrum & Wight

## UNITED STATES PATENT OFFICE

2,356,456

## SHOCK-ABSORBING OR CUSHIONING MATERIAL MADE FROM FIBROUS SUBSTANCES

Walter Garner, Menston, in Wharfedale, England,  
assignor of one-half to Lister and Company,  
Limited, Bradford, Yorkshire, England

Application August 9, 1943, Serial No. 498,005  
In Great Britain April 2, 1942

## 15 Claims.

(Cl. 28—80)

This invention relates to improvements in shock-absorbing or cushioning material made from fibrous substances.

The expression "fibrous substances" includes any mineral, protein, cellulosic or synthetic material in the form of fibres, especially fibres of an average diameter less than 500 micromillimetres and preferably less than 100 micromillimetres. Examples of such fibres are wool, cotton, mohair, kapok, glass fibre, asbestos, metal and rayon, and preferably those fibres which are inherently springy and resilient such as mohair. When fibres are used which do not inherently possess the desired degree of resilient flexibility, they may be treated, e. g. by impregnation with synthetic resin, e. g. phenol formaldehyde resin, so as to impart or augment such property.

Broadly stated, the basic feature of shock absorbing or cushioning material according to the invention is that it comprises two or more units held or secured in superposition, and each unit comprising as component elements two textile fabrics into which are woven resiliently flexible textile elements which connect the fabrics together and provide "legs" between the fabrics which, due to their length, their substantial inclination, or approach to normality, to the surfaces of the fabrics and their resistance to collapse, are capable of holding the fabrics spaced apart by at least  $\frac{1}{2}$  inch or, if external compression has been applied, of restoring them to such spacing apart when the compression is released.

The maximum useful spacing of the two textile fabrics varies according to the nature of the fibres of the connecting elements. It would not exceed, say, three inches and generally would be considerably less than that. In the case of mohair, for example, it will be found that the optimum spacing, taking into account commercial and technical considerations, is from 0.1 to 0.4 inch.

The unit fabrication may be produced, for example, in one operation on a loom capable of weaving a "warp pile" fabric (to the uncut stage), such as a "double plush" loom, which weaves for subsequent separation by cutting in the manufacture of plush, two distinct textile fabrics, preferably light in weight, tied together or connected by the "pile." Other looms which enable the connecting elements to be inserted in the form of weft may also be employed.

The resilient connecting legs may be disposed in strips, e. g. 2" wide separated by a gap of say  $\frac{1}{4}$ " wide, in order, for example, to lighten the fabrication without substantially impairing its resilience.

By employing as the connecting legs, textile elements or yarns (e. g. a two-fold yarn) which are resiliently flexible or comparatively rigid in character, and closely packing them if required, there is imparted to the fabrication a substantial springy resistance to compression which renders it suitable for use as a shock-absorbing or cushioning element which may be cut to any size or shape according to the particular purpose of its 10 application in use. Thus, for example, it may be used as a substitute for soft or sponge rubber sheets in the manufacture of seating, or other articles, or as a mattress or mattress component.

The closeness of the packing of the connecting 15 legs required for obtaining any particular degree of resiliency with a particular kind of fibre, will depend of course on the count of the yarn. By way of example it may be indicated that a satisfactory degree of resiliency may be obtained by using 1000, or between 500 and 2000, "legs" or elements per square inch of 2/32's mohair yarn, or by using 500, or between 250 and 1000, legs per square inch of 2/16's mohair yarn. It may be stated therefore that a more open spacing than 25 corresponds to 300 or 400 legs per square inch of 2/32's yarn would not be satisfactory.

The holding or securing together in superposition of the fabricated units may be effected by means of adhesive, stitching or other positive 30 methods of fastening, or in some cases the units may be held in superposition, without being attached together, by encircling or encasing means.

The fibres or yarns employed in the weaving of the unit fabrications may have been treated to 35 impart desired properties such as fire-resisting and water repelling. Alternatively, or in addition, the units themselves may be subjected to such treatment.

One or both of the outer fabrics of the units or 40 of the composite structure may be covered or interwoven with other materials having regard to the particular purpose and nature of the employment of the fabrication, or merely for decorative purposes.

45 Figures 1, 2 and 3 of the accompanying schematic drawing show, by way of example, three forms of unit fabrication which may be used in the production of shock-absorbing or cushioning material according to the invention.

50 In the drawing, 1 and 2 represent the ground warp of one outer fabric of a unit, and 3 and 4 represent the ground warp of the other outer fabric of the unit. The weft picks in the respective outer fabrics are shown in section as 5 and 6.

55 In Figure 1, which represents a standard weave,

the connecting elements or legs are produced by weaving in a "pile" yarn 1 to engage all the weft picks of both outer fabrics.

In Figure 2, which represents a derivative of the standard weave, the connecting elements or legs are produced by weaving in the "pile" yarn 1 to engage alternate weft picks in the respective outer fabrics.

In Figure 3, which represents a further derivative, the connecting elements or legs are produced by weaving in two "pile" yarns 1 as shown.

What I claim is:

1. Shock-absorbing material made from fibrous substances and comprising a plurality of units held together in superposition; and each unit comprising as component elements two textile fabrics into which are woven resiliently flexible textile elements which connect the fabrics together and provide "legs" between the fabrics which are capable of holding the fabrics spaced apart by at least  $\frac{1}{2}$  inch and, if external compression has been applied, of restoring them to such spacing apart when the compression is released.

2. Shock-absorbing material as claimed in claim 1, in which the packing of the connecting elements is at least as close as corresponds to 300 elements of  $2/32$ 's yarn per square inch.

3. Shock-absorbing material as claimed in claim 1, in which the fibres of the connecting elements of a unit are mohair and the spacing of the two textile fabrics is from 0.1 to 0.4 inch.

4. Shock-absorbing material as claimed in claim 1, in which the spacing of the two textile fabrics is from 0.1 to 0.4 inch and in which the connecting elements are  $2/32$ 's mohair yarn packed to the extent of between 500 and 2000 elements per square inch.

5. Shock-absorbing material as claimed in claim 1, in which the spacing of the two textile

fabrics is from 0.1 to 0.4 inch and in which the connecting elements are  $2/16$ 's mohair yarn packed to the extent of between 250 and 1000 elements per square inch.

5. Shock-absorbing material as claimed in claim 1, in which resilient flexibility in the fibres of the connecting elements of a unit is imparted by a treatment such as impregnation with synthetic resin.

10. Shock-absorbing material as claimed in claim 1, in which a unit fabrication has been produced in one operation on a loom capable of weaving a "warp pile" fabric to the uncut stage.

15. Shock-absorbing material as claimed in claim 1, in which the connecting elements of a unit are disposed in strips.

9. Shock-absorbing material as claimed in claim 1, in which the fibrous substance has been treated to impart fire resistance.

10. Shock-absorbing material as claimed in claim 1, in which the fibrous substance has been treated to impart water repellency.

11. Shock-absorbing material as claimed in claim 1, in which an outer fabric of a unit is covered with other material.

12. Shock-absorbing material as claimed in claim 1, in which an outer fabric of a unit is interwoven with other material.

13. Shock-absorbing material as claimed in claim 1, in which the units are positively secured together.

14. Shock-absorbing material as claimed in claim 1, in which the units are held in superposition, without being attached together, by encircling means.

15. Seats, mattresses, mattress components and other articles of manufacture comprising shock-absorbing material as claimed in claim 1.

40

WALTER GARNER.